# EUROPEAN PATENT SPECIFICATION

(11) **EP 1 177 338 B1**
(45) Date of publication and mention of the grant of the patent: **06.07.2005**
(21) Application number: 00923551.6
(22) Date of filing: 20.04.2000
(51) Int. Cl.: D01F 8/14, D04H 3/14

(54) **STRETCHABLE NONWOVEN MATERIAL**
DEHNBARER VLIESSTOFF
MATERIAU NON TISSE ETIRABLE

(30) Priority: 30.04.1999 US 303805
(43) Date of publication of application: 06.02.2002
(73) Proprietor: KIMBERLY-CLARK WORLDWIDE, INC., Neenah, Wisconsin 54956 (US)
(72) Inventor: HANCOCK-COOKE, Catherine, Marguerite, Neenah, WI 54956 (US); NEELY, James, Richard, Alpharetta, GA 30202 (US)
(74) Representative: Grünecker, Kinkeldey, Stockmair & Schwanhäusser Anwaltssozietät
(86) International application number: PCT/US2000/010705
(87) International publication number: WO 2000/066821

(56) References cited:
- EP-A- 0 317 646
- EP-A- 0 757 127
- EP-A- 0 905 292
- US-A- 5 814 569

## Description

This invention relates to a nonwoven material which exhibits elastomeric properties although containing no thermoplastic elastomers or rubbers. More particularly, this invention relates to a nonwoven material that is stretchable in a machine direction and/or a cross direction without the use of thermoplastic elastomers or rubbers. The nonwoven material exhibits elastic recovery in both the machine direction and the cross direction when stretched up to about 30%. The material is particularly suitable for use in personal care absorbent articles such as diapers, training pants and adult incontinence garments.

Absorbent personal care articles such as sanitary napkins, disposable diapers, incontinent-care pads and the like are widely used, and much effort has been made to improve the effectiveness and functionalities of these articles. Thick, flat personal care articles of the past that do not fit the shape of the human body and do not conform to the movements of the user have been largely replaced by resiliently conforming 3-dimensional, body-shaped articles.

Nonwoven webs are defined as webs having a structure of individual fibers or threads which are interlaid, but not in a regular or identifiable manner, as in a knitted fabric. Nonwoven webs can be formed by many processes such as, for example, meltblowing processes, spunbonding processes, and bonded carded web processes. Typically, the fibers from these processes are deposited onto a forming wire or belt for formation of the web. When subjected to heat following formation of the web, there is a tendency for the nonwoven web to shrink. Shrinkage of the nonwoven web is considered to be disadvantageous in that it generally results in non-uniformity of the web. See for example, U.S. Patent 5,382,400 and U.S. Patent 5,418,045, both to Pike et al., which teach a process for making nonwoven polymeric fabrics wherein continuous meltspun multicomponent polymeric filaments are crimped before the continuous multicomponent filaments are formed into a nonwoven web, resulting in a substantial reduction in shrinkage and a substantially stable and uniform nonwoven web.
US Patent 5,814,569 discloses a nonwoven fabric of superior uniaxial elasticity, comprising conjugate filaments, each of which is concentric sheath-core type.

It will be apparent, however, that diapers, training pants and incontinence garments made from substantially stable, uniform nonwoven webs may not conform to the movement of the wearer, reducing the comfort, and possibly the functionality, of the articles. To date, as indicated hereinabove, this issue has been addressed by resiliently conforming 3-dimensional, body-shaped articles as well as articles employing elastic films.

It is one object of this invention to provide a nonwoven web material which exhibits elastic properties, and to provide a nonwoven web material which exhibits elastic properties and which does not employ any thermoplastic elastomers or rubbers.
The object of the invention is achieved by a stretchable nonwoven material comprising:
- a nonwoven web comprising a plurality of bicomponent fibers comprising a polyester and a second polymer, said nonwoven web having been bonded by a method selected from the group consisting of pattern-bonding, point-bonding and combinations thereof and then heated,
- wherein said polyester is a polyester that shrinks upon being heated,
   and said second polymer is a polymer that shrinks less than said polyester upon being heated, and
- wherein said bicomponent fibers are configured such that both of said polyester and said second polymer are present on a surface of said fibers.

It is preferred that said polyester is polyethylene terephthalate.
It is also preferred that said bicomponent fibers are configured as one of a side-by-side, polylobal, and pie arrangement.
Moreover it is preferred that said polyester comprises in a range of about 20% to about 90% by weight of said bicomponent fibers.
It is also preferred that said polyester comprises in a range of about 40% by weight to about 65% by weight of said bicomponent fibers.
Further, it is preferred that said bicomponent fibers are spunbond.
Moreover, it is preferred that said second polymer is a polymer selected from the group consisting of polyolefins and polyamides.
More preferably, said second polymer is selected from the group consisting of polyethylene, polypropylene and nylon.
It is also preferred that said bicomponent fibers are splittable.
Said object is also achieved by a method for producing a stretchable nonwoven material comprising the steps of:
- forming a nonwoven web using a plurality of bicomponent fibers, said bicomponent fibers comprising a polyester and a second polymer, wherein the polyester shrinks upon being heated and the second polymer does not shrink as much as the polyester upon heating, wherein said bicomponent fibers are configured such that both of said polyester and said second polymer are present on a surface of said fibers,
- bonding said nonwoven web using a method selected from the group consisting of pattern-bonding, point-bonding and combinations thereof; and
- heating said nonwoven web, resulting in a stretchable nonwoven web.

It is preferred that said polyester is polyethylene terephthalate.
It is also preferred that said second polymer is a polymer selected from the group consisting of polyolefins and polyamides.
It is furthermore preferred that said bicomponent fibers are spunbond.
Moreover, it is preferred that said polyester comprises in a range of about 20% by weight to about 90% by weight of said bicomponent fibers
Additionaly, it is preferred that said polyester comprises in a range of about 40% to about 65% by weight of said bicomponent fibers.
Preferably, said bicomponent fibers are configured as one of a side-by-side, polylobal and pie arrangement.
More preferably, said polyolefin is selected from the group consisting of polyethylene and polypropylene.
It is also preferred that said polyamide is nylon.

Said object is further achieved by a personal care article comprising:
- a nonwoven web comprising a plurality of bicomponent fibers comprising a polyester and a second polymer, wherein the polyester shrinks upon being heated and the second polymer does not shrink as much as the polyester upon heating, wherein said bicomponent fibers are configured such that both of said polyester and said second polymer are present on a surface of said fibers,
- said nonwoven web having been bonded by a method selected from the group consisting of pattern-bonding, point-bonding and combinations thereof, and then heated after formation.

Suitable polyesters for use in this invention are any polyesters which shrink upon being heated. In accordance with one particularly preferred embodiment, the polyester is polyethylene terephthalate (PET). The second polymer is one which does not shrink as much as the polyester upon heating, preferably a polyolefin or a polyamide. The resulting stretchable nonwoven material is stretchable up to about 30% of its unbiased length in the machine direction and/or the cross machine direction. Upon release of the bias force, the nonwoven material exhibits elastic recovery in both the machine direction and the cross direction, returning substantially to its original dimensions. Depending upon the polyester and second polymer used to form the fibers, the fibers can be made to split.

### BRIEF DESCRIPTION OF THE DRAWINGS

These and other objects and features of this invention will be better understood from the following detailed description taken in conjunction with the drawings wherein:
Fig. 1 is a schematic diagram of a process line for producing a stretchable nonwoven material in accordance with this invention; and
Fig. 2 is a table showing the results obtained from materials produced in accordance with the method of this invention.

The term "stretchable" is used herein to mean any material which, upon application of a biasing force, is elongatable, to a stretched, bias length and which will recover at least 50% of its elongation upon release of the stretching, elongating force. A hypothetical example would be a one (1) inch sample of a material which is elongatable to at least 3.81 cm (1.50 inches) (50% elongation) and which, upon being elongated to 3.81 cm (1.50 inches) and released, will recover to a length of not more than 3.175 cm (1.25) (50% recovery) inches.

As used herein, the term "nonwoven web" or "nonwoven material" means a web having a structure of individual fibers or threads which are interlaid, but not in a regular or identifiable manner, as in a knitted fabric and films that have been fibrillated. Nonwoven webs or materials have been formed from many processes such as, for example, meltblowing processes, spunbonding processes, and bonded carded web processes. The basis weight of nonwoven webs or materials is usually expressed in ounces of material per square yard (osy) or grams per square meter (gsm), and the fiber diameters usable are usually expressed in microns. (Note that to convert from osy to gsm, multiply osy by 33.91.)

As used herein, the term "spunbond fibers" refers to small diameter fibers which are formed by extruding molten thermoplastic material as filaments from a plurality of fine, usually circular capillaries of a spinneret with a diameter of the extruded filaments then being rapidly reduced as taught, for example, by U.S. Patent 4,340,563 to Appel et al., U.S. Patent 3,692,618 to Dorschner et al., U.S. Patent 3,802,817 to Matsuki et al., U.S. Patent 3,338,992 and U.S. Patent 3,341,394 to Kinney, U.S. Patent 3,502,763 to Hartmann, U.S. Patent 3,502,538 to Levy, and U.S. Patent 3,542,615 to Dobo et al. Spunbond fibers are quenched and generally not tacky when they are deposited onto a collecting surface. Spunbond fibers are generally continuous and have average diameters larger than 7 microns, more particularly, between about 10 and 35 microns.

As used herein, the term "meltblown fibers" refers to fibers formed by extruding a molten thermoplastic material through a plurality of fine, usually circular, die capillaries as molten threads or filaments into converging high velocity gas streams (for example, airstreams) which attenuate the filaments of molten thermoplastic material to reduce their diameter, which may be to microfiber diameter. Thereafter, the meltblown fibers are carried by the high velocity gas stream and are deposited on a collecting surface to form a web of randomly dispersed meltblown fibers. Such a process is disclosed, for example, by U.S. Patent 3,849,241 to Butin. Meltblown fibers are microfibers which may be continuous or discontinuous, are generally smaller than 10 microns in average diameter, and are generally tacky when deposited onto a collecting surface.

As used herein, the term "bonded carded web" refers to webs made from staple fibers which are sent through a combing or carding unit, which breaks apart and aligns the staple fibers in the machine direction to form a generally machine direction-oriented fibrous nonwoven web. Such fibers are usually purchased in bales which are placed in a picker which separates the fibers prior to the carding unit. Once the web is formed, it is then bonded by one or more of several known bonding methods.

As used herein, the term "microfibers" refers to small diameter fibers having an average diameter not greater than about 75 microns, for example, having an average diameter of from about 0.5 microns to about 50 microns, or more particularly, having an average diameter of from about 2 microns to about 40 microns. Another frequently used expression of fiber diameter is denier, which is defined as grams per 9000 meters of a fiber, and may be calculated as fiber diameter in microns squared, multiplied by the density in grams/cc, multiplied by 0.00707. A lower denier indicates a finer fiber and a higher denier indicates a thicker or heavier fiber. For example, a diameter of a polypropylene fiber given as 15 microns may be converted to denier by squaring, multiplying the results by 0.89 g/cc and multiplying by 0.00707. Thus, a 15 micron polypropylene fiber has a denier of about 1.42. Outside the United States, the unit of measurement is more commonly the "tex", which is defined as the grams per kilometer of fiber. Tex may be calculated as denier/9.

As used herein, the term "polymer" generally includes, but is not limited to, homopolymers, copolymers, such as, for example, block, graft, random and alternating copolymers, terpolymers, etc., and blends and modifications thereof. Furthermore, unless otherwise specifically limited, the term "polymer" also includes all possible geometric configurations of the material. These configurations include, but are not limited to, isotactic, syndiotactic, atactic and random symmetries.

As used herein, the term "personal care article" means disposable diapers, training pants, absorbent underpants, adult incontinence products, and feminine hygiene products.

As used herein, the term "bicomponent fibers" refers to fibers which have been formed from at least two polymers extruded from separate extruders but spun together to form one fiber. Bicomponent fibers are also sometimes referred to as conjugate fibers or multicomponent fibers. The polymers are arranged in substantially constantly positioned distinct zones across the cross-sections of the bicomponent fibers and extend continuously along the length of the bicomponent fibers. The configuration of such a bicomponent fiber may be, for example, a sheath/core arrangement wherein one polymer is surrounded by another, or may be a side-by-side arrangement, a pie arrangement, or an "islands-in-the-sea" arrangement. Bicomponent fibers are taught by U.S. Patent 5,108,820 to Kaneko et al., U.S Patent 4,795,668 to Krueger et al., U.S. Patent 5,540,992 to Marcher et al., and U.S. Patent 5,336,552 to Strack et al Bicomponent fibers are also taught by U.S. Patent 5,382,400 to Pike et al. For two component fibers, the polymers may be present in ratios of 75/25, 50/50, 25/75 or any other desired ratio.

As used herein, the term "machine direction" or "MD" means the length of a fabric in the direction in which it is produced. The term "cross machine direction" or "CD" means the width of fabric, that is a direction generally perpendicular to the MD.

As used herein, the term "consisung essentially of" does not exclude the presence of additional materials which do not significantly affect the desired characteristics of a given composition or product. Exemplary materials of this sort would include, without limitation, pigments, annoxidants, stabilizers, surfactants, waxes, flow promoters, solvents, particulates, and materials added to enhance procsssability of the composition.

The invention disclosed herein is a nonwoven material that exhibits elastomeric properties although it contains no thermoplastic elastomers or rubbers. The material comprises a nonwoven web made of bicomponent fibers containing a polyester and a second polymer, such as polyethylene. When the web is pattern-bonded or point-bonded and exposed to a heating process subsequent to being bonded, it shrinks, resulting in a nonwoven material that exhibits elastic recovery in both the machine direction and the cross direction when stretched up to about 30%. The nonwoven web is preferably heated to a temperature of at least about 104.4 °C (220°F). The amount of stretch and recovery is adjustable by varying the "shrinkage" temperature, and/or bond area and/or polyester content. In addition, the amount of shrinkage increases as the basis weight of the nonwoven web increases.

Fig. 1 is a schematic diagram of a process line for producing a stretchable nonwoven material in accordance with this invention. The process line 10 is arranged to produce bicomponent continuous filaments. The process line 10 includes a pair of extruders 12a and 12b for separately extruding a polymer component A, a polyester in the instant case, and a polymer component B, for example a polyolefin. Polymer A is fed into the respective extruder 12a from a first hopper 14a and polymer component B is fed into the respective extruder 12b from a second hopper 14b. Polymer components A and B are fed from extruders 12a and 12b through respective polymer conduits 16a and 16b to a spinneret 18. Spinnerets are well known to those skilled in the art and, thus, will not be described in detail herein. Generally, the spinneret 18 includes a housing containing a spin pack which includes a plurality of plates stacked one on top of the other with a pattern of openings arranged to create flow paths for directing polymer A and polymer B separately through the spinneret. The spinneret 18 has openings arranged in one or more rows. The spinneret openings form a downwardly extending curtain of filaments when the polymers are extruded through the spinneret. For purposes of the present invention, the spinneret 18 is arranged so as to form bicomponent filaments wherein both polymer A and polymer B are disposed on a portion of the surface thereof. Such bicomponent filaments include side-by-side arrangements, pie arrangements and polylobal arrangements in which one of the polymers forms at least a portion of the lobes, which lobes are disposed at a distance from one another, and the second polymer is centrally disposed, at least a portion of the surface of which can be seen in the area between the lobes.

The process line 10 also includes a quench blower 20 positioned adjacent to the curtain of filaments extending from spinneret 18. Air from the quench air blower 20 quenches the filaments extending from spinneret 18.

A fiber draw unit or aspirator 22 is disposed below spinneret 18 and receives the quenched filaments. Fiber draw units or aspirators for use in meltspinning polymers are well known to those skilled in the art. Suitable fiber draw units for use in this process include a linear fiber aspirator of the type shown in U.S. Patent 3,802,817 and eductive guns of the type shown in U.S. Patents 3,692,618 and 3,423,266.

Generally described, fiber draw unit 22 includes an elongated vertical passage through which the filaments are drawn, aspirating air entering from the sides of the passage and flowing downward through the passage. Heater 24 supplies hot aspirating air to fiber draw unit 22. The hot aspirating air draws the filaments and ambient air through fiber draw unit 22.

An endless foraminous forming surface 26 is positioned below fiber draw unit 22 and receives the continuous filaments from the outlet opening of fiber draw unit 22. The forming surface 26 travels around guide rollers 28. A vacuum 30 positioned below the forming surface 26 where the filaments are deposited draws the filaments against the forming surface.

The process line 10 further compnses compression roller 32 which, along with the forwardmost of the guide rollers 28, receive the web as it is drawn off of the forming surface 26. In addition, process line 10 further includes a bonding apparatus such as pattern bonding, or thermal point bonding, 34.

Thermal point bonding involves passing a fabric or web of fibers to be bonded between a heated calender roll and an anvil roll. The calender roll is usually, though not always, patterned in some way so that the entire fabric is not bonded across its entire surface. As a result, various patterns for calender rolls have been developed for functional as well as aesthetic reasons. One example of a pattern has points and is the Hansen Pennings or "H&P" pattern with about a 30% bond area with about 200 bonds 6.54 cm² (square inch) as taught in U.S. Pat. No. 3,855,046 to Hansen and Pennings. The H&P pattern has square point or pin bonding areas wherein each pin has a side dimension of 0.038 inches (0.965 mm), a spacing of 0.070 inches (1.778 mm) between pins, and a depth of bonding of 0.023 inches (0.584 mm). The resulting pattern has a bonded area of about 29.5%. Another typical point bonding pattern is the expanded Hansen and Pennings or "EHP" bond pattern which produces a 15% bond area with a square pin having a side dimension of 0.037 inches (0.94 mm), a pin spacing of 0.097 inches (2.464 mm) and a depth of 0.039 inches (0.991 mm). Another typical point bonding pattern designated "714" has square pin bonding areas wherein each pin has a side dimension of 0.584 mm (0.023 inches), a spacing of 0.062 inches (1.575 mm) between pins, and a depth of bonding of 0.033 inches (0.838 mm). The resulting pattern has a bonded area of about 15%. Yet another common pattern is the C-Star pattern which has a bond area of about 16.9%. The C-Star pattern has a cross-directional bar or "corduroy" design interrupted by shooting stars. Other common patterns include a diamond pattern with repeating and slightly offset diamonds and a wire weave pattern looking as the name suggests, e.g., like a window screen.

Downstream of thermal point bonding rollers 34 is a hot air knife 36, or some other heating process, such as an oven, for heating the web to a desired temperature. A conventional hot air knife includes a mandrel with a slot that blows a jet of hot air onto the nonwoven web surface. Such hot air knives are taught, for example, by U.S. Patent 4,567,796 to Kloehn et al. Alternatively, the material can be laundered, is washed and dried at elevated temperatures to obtain the desired shrinkage.

As previously indicated, the nonwoven web used to make the nonwoven material of this invention comprises a plurality of bicomponent fibers containing a polyester and a second polymer, such as polyethylene. Although any polyester that shrinks upon heating may be used, in accordance with one particularly preferred embodiment, the polyester is polyethylene terephthalate. The second polymer comprising the bicomponent fibers is a polymer selected from the group consisting of polyolefins and polyamides. Particularly preferred polyolefins are polyethylene and polypropylene. Suitable polyamides include, but are not limited to, nylon 6, nylon 6/6, nylon 10, nylon 12 and the like.

Depending upon the selection of the polyester and the second polymer used to form the bicomponent fibers, the fibers can be rendered splittable, thereby enhancing the softness of nonwoven materials produced from them. These fibers can be split by any number of mechanical, thermal or chemical means. And, although splitting of the bicomponent fibers is not required for shrinkage of the nonwoven web during formation and for elastomeric recovery of the formed nonwoven web, it may increase the elastomeric characteristics of the material.

In accordance with one preferred embodiment of this invention, the bicomponent filament comprises in a range of about 40% by weight to about 90% by weight of polyester (PET). In accordance with a particularly preferred embodiment of this invention, the bicomponent filament comprises in a range of about 55% by weight to about 65% by weight of polyester.

The stretchable nonwoven material of this invention in accordance with one embodiment of this invention comprises bicomponent filaments which are produced by a bonded carded web process. In accordance with a particularly preferred embodiment, the bicomponent filaments used to produce the nonwoven web are spunbonded.

### Examples

Fig 2 is a summary of data collected in connection with stretchable nonwovens produced in accordance with the method of this invention. Data is presented for five sample materials produced from side-by-side bicomponent fibers of PET and low linear density polyethylene, samples numbered 1-5. Two sets of data are presented for each sample - machine direction (MD) stretchability and cross direction (CD) stretchability. Process condinons for preparation of these samples were as follows:
Polymers:
   PET= Ticona EKX-183
   LLDPE= Dow 6811 A
   HDPE= Dow 25455
Hole Diameter = 0.6 mm
Throughput = 0.6 ghm
Melt Temperature = 525°
Quench Air Temp = (61 °F) 16.1 °C
Polymer Ratio = 50/50 (by volume) or 59/41 PET/PE (by weight)
Bond Pattern = see examples (5% and 10% spirals, and HP)

Data for a 16 piece splittable pie configured bicomponent fiber nonwoven web, Sample 6, is also presented. In this case the bicomponent fibers were produced from PET and high density polyethylene (HDPE).

## Claims

1. A stretchable nonwoven material comprising:
- a nonwoven web comprising a plurality of bicomponent fibers comprising a polyester and a second polymer, said nonwoven web having been bonded by a method selected from the group consisting of pattern-bonding, point-bonding and combinations thereof and then heated,
- wherein said polyester is a polyester that shrinks upon being heated,
and said second polymer is a polymer that shrinks less than said polyester upon being heated, and
- wherein said bicomponent fibers are configured such that both of said polyester and said second polymer are present on a surface of said fibers.

2. A stretchable nonwoven material in accordance with claim 1, wherein said polyester is polyethylene terephthalate.

3. A stretchable nonwoven material in accordance with claim 1, wherein said bicomponent fibers are configured as one of a side-by-side, polylobal, and pie arrangement.

4. A stretchable nonwoven material in accordance with claim 1, wherein said polyester comprises in a range of 20% to 90% by weight of said bicomponent fibers.

5. A stretchable nonwoven material in accordance with claim 1, wherein said polyester comprises in a range of 40% by weight to 65% by weight of said bicomponent fibers.

6. A stretchable nonwoven material in accordance with claim 1, wherein said bicomponent fibers are spunbond.

7. A stretchable non-woven material in accordance with claim 1, wherein said second polymer is a polymer selected from the group consisting of polyolefins and polyamides.

8. A stretchable nonwoven material in accordance with claim 7, wherein said second polymer is selected from the group consisting of polyethylene, polypropylene and nylon.

9. A stretchable nonwoven material in accordance with claim 1, wherein said bicomponent fibers are splittable.

10. A method for producing a stretchable nonwoven material comprising the steps of:
- forming a nonwoven web using a plurality of bicomponent fibers, said bicomponent fibers comprising a polyester and a second polymer, wherein the polyester shrinks upon being heated and the second polymer does not shrink as much as the polyester upon heating, wherein said bicomponent fibers are configured such that both of said polyester and said second polymer are present on a surface of said fibers,
- bonding said nonwoven web using a method selected from the group consisting of pattern-bonding, point-bonding and combinations thereof; and
- heating said nonwoven web, resulting in a stretchable nonwoven web.

11. A method in accordance with claim 10, wherein said polyester is polyethylene terephthalate.

12. A method in accordance with claim 10, wherein said second polymer is a polymer selected from the group consisting of polyolefins and polyamides.

13. A method in accordance with claim 10, wherein said bicomponent fibers are spunbond.

14. A method in accordance with claim 10, wherein said polyester comprises in a range of 20% by weight to 90% by weight of said bicomponent fibers.

15. A method in accordance with claim 10, wherein said polyester comprises in a range of 40% to 65% by weight of said bicomponent fibers.

16. A method in accordance with claim 10, wherein said bicomponent fibers are configured as one of a side-by-side, polylobal and pie arrangement.

17. A method in accordance with claim 12, wherein said polyolefin is selected from the group consisting of polyethylene and polypropylene.

18. A method in accordance with claim 12, wherein said polyamide is nylon.

19. A personal care article comprising:
- a nonwoven web comprising a plurality of bicomponent fibers comprising a polyester and a second polymer, wherein the polyester shrinks upon being heated and the second polymer does not shrink as much as the polyester upon heating, wherein said bicomponent fibers are configured such that both of said polyester and said second polymer are present on a surface of said fibers,
- said nonwoven web having been bonded by a method selected from the group consisting of pattern-bonding, point-bonding and combinations thereof, and then heated after formation.

## Patentansprüche

1. Ein dehnbarer Vliesstoff, umfassend
- ein Vlies- Netz umfassend eine Vielzahl von Zwei- Komponenten- Fasern umfassend einen Polyester und ein zweites Polymer, wobei besagtes Vliesnetz durch ein Verfahren verbunden wurde, ausgewählt aus der Gruppe bestehend aus Muster- Verknüpfung, Punkt- Verknüpfung und Kombinationen davon und anschließend erhitzt wurde,
- wobei besagter Polyester ein Polyester ist, welcher sich bei Erhitzung zusammenzieht, und besagtes zweites Polymer ein Polymer ist, das sich weniger als besagter Polyester beim Erhitzen zusammenzieht und
- wobei besagte Zwei- Komponenten- Fasern so konfiguriert sind, dass sowohl besagter Polyester als auch besagtes zweites Polymer auf der Oberfläche von besagten Fasern vorliegen.

2. Ein dehnbarer Vliesstoff in Übereinstimmung mit Anspruch 1, wobei besagter Polyester Polyethylenterephthalat ist.

3. Ein dehnbarer Vliesstoff in Übereinstimmung mit Anspruch 1, wobei besagte Zwei- Komponenten- Fasern konfiguriert als eines von nebeneinander, polylobal oder einer Torten- Anordnung konfiguriert sind.

4. Ein dehnbarer Vliesstoff in Übereinstimmung mit Anspruch 1, wobei besagter Polyester in einem Bereich von 20 Gew. - % bis 90 Gew. - % von besagten ZweiKomponenten- Fasern umfasst.

5. Ein dehnbarer Vliesstoff in Übereinstimmung mit Anspruch 1, wobei besagter Polyester in einem Bereich von 40 Gew.- % bis 65 Gew.- % von besagten ZweiKomponenten- Fasern umfasst.

6. Ein dehnbarer Vliesstoff in Übereinstimmung mit Anspruch 1, wobei gesagte Zwei- Komponenten- Fasern spinngebunden sind.

7. Ein dehnbarer Vliesstoff in Übereinstimmung mit Anspruch 1, wobei besagtes zweites Polymer ein Polymer ist, ausgebildet aus der Gruppe bestehend von Polyolefinen und Polyamiden.

8. Ein dehnbarer Vliesstoff in Übereinstimmung mit Anspruch 7, wobei gesagtes zweites Polymer ausgewählt aus der Gruppe bestehend aus Polyethylen, Polypropylen und Nylon ist.

9. Ein dehnbarer Vliesstoff in Übereinstimmung mit Anspruch 1, wobei besagte Zwei- Komponenten- Fasern spaltbar sind.

10. Ein Verfahren zum Herstellen eines dehnbaren Vliesstoffes umfassend die Schritte von:
- Ausbilden eines Vlies- Netzes unter Verwendung einer Vielzahl von ZweiKomponenten- Fasern, wobei besagte Zwei- Komponenten- Fasern einen Polyester und ein zweites Polymer umfassen, wobei der Polyester sich zusammenzieht beim Erhitzen und das zweite Polymer sich nicht in dem Maße, wie das Polyester beim Erhitzen zusammenzieht, wobei besagte Zwei- Komponenten- Fasern so konfiguriert sind, dass beide, besagter Polyester und besagtes Polymer, auf der Oberfläche von besagten Fasern vorliegen,
- Verknüpfen besagten Vlies- Netzes unter Verwendung eines Verfahrens ausgewählt aus der Gruppe bestehend aus Muster- Verknüpfung, Punkt-Verknüpfung und Kombinationen davon; und
- Erhitzen besagten Vlies- Netzes resultierend in einem dehnbaren VliesNetz.

11. Ein Verfahren gemäß Anspruch 10, wobei besagter Polyester Polyetylentherephthalat ist.

12. Ein Verfahren in Übereinstimmung mit Anspruch 10, wobei besagtes zweites Polymer ein Polymer ist ausgebildet aus der Gruppe bestehend aus Polyolefinen und Polyamiden.

13. Ein Verfahren in Übereinstimmung mit Anspruch 10, wobei besagte ZweiKomponenten- Fasern spinngebunden sind.

14. Ein Verfahren in Übereinstimmung mit Anspruch 10, wobei besagter Polyester in einer Größenordnung von 20 Gew.- % bis 90 Gew.- % von besagten ZweiKomponenten- Fasern umfasst.

15. Ein Verfahren in Übereinstimmung mit Anspruch 10, wobei besagter Polyester in einer Größenordnung von ungefähr 40 Gew.- % bis 65 Gew.- % von besagten Zwei- Komponenten- Fasern umfasst.

16. Ein Verfahren in Übereinstimmung mit Anspruch 10, wobei besagte ZweiKomponenten- Fasern konfiguriert sind als eines von nebeneinander, polylobal, oder einer Torten- Anordnung.

17. Ein Verfahren in Übereinstimmung mit Anspruch 12, wobei besagtes Polyolefin ausgewählt ist aus der Gruppe bestehend aus Polyethylen und Polypropylen.

18. Ein Verfahren in Übereinstimmung mit Anspruch 12, wobei besagtes Polyamid Nylon ist.

19. Ein Hygieneartikel umfassend:
- ein Vlies- Netz umfassend eine Vielzahl von Zwei- Komponenten- Fasern umfassend einen Polyester und ein zweites Polymer, wobei das Polymer sich zusammenzieht beim Erhitzen und das zweite Polymer sich nicht in dem Maße, wie der Polyether beim Erhitzen zusammenzieht, wobei besagte Zwei- Komponenten- Fasern so konfigunert sind, dass sowohl besagter Polyester als auch besagtes zweites Polymer auf der Oberfläche von besagten Fasern vorliegen,
- besagtes Vlies- Netz verknüpft wurde durch ein Verfahren ausgewählt aus der Gruppe bestehend aus Muster- Verknüpfung, Punkt- Verknüpfung und Kombinationen davon und nach Ausbildung erhitzt worden ist

## Revendications

1. Matériau non-tissé extensible comprenant :
- un voile non-tissé comprenant une pluralité de fibres bicomposées comprenant un polyester et un second polymère, ledit voile non-tissé ayant été lié par une méthode sélectionnée dans le groupe consistant en la liaison selon un motif, la liaison par points et leurs combinaisons, puis chauffé,
- où ledit polyester est un polyester qui rétrécit lorsqu'il est chauffé,
et ledit second polymère est un polymère qui rétrécit moins que ledit polyester lorsqu'il est chauffé, et
- où lesdites fibres bicomposées sont configurées de telle sorte que ledit polyester et ledit second polymère sont tous deux présents sur une surface desdites fibres.

2. Matériau non-tissé extensible selon la revendication 1, dans lequel ledit polyester est le poly(téréphtalate d'éthylène).

3. Matériau non-tissé extensible selon la revendication 1, dans lequel lesdites fibres bicomposées sont configurées selon l'un des agencements côte à côte, polylobé, et en parts de tarte.

4. Matériau non-tissé extensible selon la revendication 1, dans lequel ledit polyester représente de 20 % à 90 % en poids desdites fibres bicomposées.

5. Matériau non-tissé extensible selon la revendication 1, dans lequel ledit polyester représente de 40 % en poids à 65 % en poids desdites fibres bicomposées.

6. Matériau non-tissé extensible selon la revendication 1, dans lequel lesdites fibres bicomposées sont obtenues par filage-nappage.

7. Matériau non-tissé extensible selon la revendication 1, dans lequel ledit second polymère est un polymère sélectionné dans le groupe consistant en les polyoléfines et les polyamides.

8. Matériau non-tissé extensible selon la revendication 7, dans lequel ledit second polymère est sélectionné dans le groupe consistant en le polyéthylène, le polypropylène et le nylon.

9. Matériau non-tissé extensible selon la revendication 1, dans lequel lesdites fibres bicomposées sont fendables.

10. Méthode de production d'un matériau non-tissé extensible comprenant les étapes de :
- formation d'un voile non-tissé utilisant une pluralité de fibres bicomposées, lesdites fibres bicomposées comprenant un polyester et un second polymère, où le polyester rétrécit lorsqu'il est chauffé et le second polymère ne rétrécit pas autant que le polyester lorsqu'il est chauffé, et où lesdites fibres bicomposées sont configurées de telle sorte que ledit polyester et ledit second polymère sont tous deux présents sur une surface desdites fibres,
- liaison dudit voile non-tissé en utilisant une méthode sélectionnée dans le groupe consistant en la liaison selon un motif, la liaison par points et leurs combinaisons ; et
- chauffage dudit voile non-tissé, débouchant sur un voile non-tissé extensible.

11. Méthode selon la revendication 10, dans laquelle ledit polyester est le poly(téréphtalate d'éthylène).

12. Méthode selon la revendication 10, dans laquelle ledit second polymère est un polymère sélectionné dans le groupe consistant en les polyoléfines et les polyamides.

13. Méthode selon la revendication 10, dans laquelle lesdites fibres bicomposées sont obtenues par filage-nappage.

14. Méthode selon la revendication 10, dans laquelle ledit polyester représente de 20 % en poids à 90 % en poids desdites fibres bicomposées.

15. Méthode selon la revendication 10, dans laquelle ledit polyester représente de 40 % à 65 % en poids desdites fibres bicomposées.

16. Méthode selon la revendication 10, dans laquelle lesdites fibres bicomposées sont configurées selon l'un des agencements côte à côte, polylobé et en parts de tarte.

17. Méthode selon la revendication 12, dans laquelle ladite polyoléfine est sélectionnée dans le groupe consistant en le polyéthylène et le polypropylène

18. Méthode selon la revendication 12, dans laquelle ledit polyamide est le nylon.

19. Article d'hygiène intime comprenant :
- un voile non-tissé comprenant une pluralité de fibres bicomposées comprenant un polyester et un second polymère, où le polyester rétrécit lorsqu'il est chauffé et le second polymère ne rétrécit pas autant que le polyester lorsqu'il est chauffé, et où lesdites fibres bicomposées sont configurées de telle sorte que ledit polyester et ledit second polymère sont tous deux présents sur une surface desdites fibres,
- ledit voile non-tissé ayant été lié par une méthode sélectionnée dans le groupe consistant en la liaison selon un motif, la liaison par points et leurs combinaisons, puis chauffé après formation.
